

# UNITED STATES PATENT OFFICE.

GEORGES LÉPINE, OF NEUCHATEL, SWITZERLAND.

## UNINFLAMMABLE LIQUIDS ADAPTED FOR USE IN INSULATING AND OTHER SIMILAR PURPOSES.

1,255,618.

Specification of Letters Patent.

Patented Feb. 5, 1918.

No Drawing. Original application filed April 13, 1914, Serial No. 831,618. Divided and this application filed June 29, 1917. Serial No. 177,819.

To all whom it may concern:

Be it known that I, GEORGES LÉPINE, chemist, a citizen of the Republic of France, residing at Neuchatel, Canton of Neuchatel, in the Confederation of Switzerland, have invented certain new and useful Improvements in Uninflammable Liquids Adapted for Use in Insulating and other Similar Purposes, of which the following is a specification.

This invention relates to an uninflammable liquid adapted for use in insulating and other similar purposes and is a division of my co-pending application Serial No. 831,618 filed April 13, 1914.

I am aware that heretofore it has been proposed to render partially uninflammable oil which is to be employed as an insulating material in electrical apparatus such for example, as oil break switches, transformers, and the like, by mixing the oil with uninflammable substances. By this mixture a liquid is obtained which at ordinary temperatures and up to 100° C. is not inflammable but which when heated to this or a higher temperature becomes inflammable again because the uninflammable ingredients have evaporated therefrom, and on the contrary the present invention relates to a liquid which is uninflammable in all its ingredients and forms an excellent substitute for the inflammable oil usually employed as an insulator in electrical apparatus.

This liquid made in accordance with the present invention consists preferably of pentachlorethane mixed with one or more chlorin compounds of hydrocarbons of the benzene series, such for example as trichlorobenzene,  $C_6H_5Cl_3$ , pentachlorobenzene  $C_6HCl_5$ , and hexachlorobenzene  $C_6Cl_6$ .

For example, a mixture of this compound may consist in

80 parts pentachlorethane  
18 parts pentachlorobenzene  
45 2 parts hexachlorobenzene with the addition of  
1 part toluidin.

This mixture is made as follows:

The pentachlorobenzene and the hexachlorobenzene are dissolved in the pentachlorethane and 1 per cent. toluidin is added in order to fix the bodies which owing to decomposition would be injurious to metals and would then become electric conductors, owing to the said decomposition.

By the characteristic odor of the vapors produced from this mixture, when heated, there is the advantage of indicating for example a probable perturbation of the electrical apparatus in which the liquid is employed as an insulator in substitution of the ordinary oil. This mixture when gradually heated in an open crucible until vapors evolve does not take fire even when the flame is directed into the vapor, but on the contrary these vapors extinguish the flame. Tests have been made for determining the dielectric properties of this mixture and these show the following results:

The electric puncture test has been made between two points immersed in the liquid at 18° C. The spark distance between the two points varied from 2.5 to 10 mm. and the tension was gradually raised until the first spark occurred. The tension was supplied by a transformer of 20 k. w. of 100000 volts at 50 cycles per second.

The following are some values of tensions at which the first spark occurred:

| Spark distance. | Minimal volts. | Maximal volts. | Mean of 6 punctures. |
|-----------------|----------------|----------------|----------------------|
| mm.             |                |                | Volts.               |
| 2.5.....        | 11,600         | 16,100         | 18,650               |
| 5.0.....        | 22,000         | 22,500         | 22,800               |
| 10.0.....       | 36,900         | 44,600         | 41,000               |

I claim as my invention:

1. An uninflammable and insulating liquid comprising a mixture of pentachlorethane and a chlorin compound of the hydrocarbons of the benzene series together with the addition of a material to prevent the decomposition of the liquid.

2. An uninflammable and insulating liquid comprising a mixture of pentachlorethane, pentachlorobenzene and toluidin.
3. An uninflammable and insulating liquid comprising a mixture of pentachlorethane, pentachlorobenzene, hexachlorobenzene and toluidin.
4. An uninflammable and insulating liquid comprising a mixture of

10 80 parts pentachlorethane

18 parts pentachlorobenzene  
2 parts hexachlorobenzene with the addition of one part toluidin.  
In testimony whereof I have affixed my signature in presence of two witnesses.

GEORGES LÉPINE.

Witnesses:

A. J. LIERNUR,  
ROB. DE WURSTEMBERG.